

## UNITED STATES PATENT OFFICE

2,247,569

## PROCESS OF HARDENING AND SIMULTANEOUSLY INCREASING THE SENSITIVITY OF PHOTOGRAPHIC SILVER HALIDE EMULSIONS

Johannes Brunken, Dessau-Ziebigk, and Hans Fricke and Gustav Wilmanns, Wolfen, Kreis Bitterfeld, Germany, assignors to General Aniline & Film Corporation, New York, N. Y., a corporation of Delaware

No Drawing. Application February 28, 1940, Serial No. 321,208. In Germany February 9, 1939

4 Claims. (Cl. 95—7)

This invention relates to hardening and simultaneously increasing the sensitivity of photographic silver halide emulsions. Aldehydes and ketones, for instance formaldehydes, glyoxal, oxyketones, are generally used for the hardening of photographic emulsions. All of these hardening agents however show the disadvantage to continue the hardening process later on during storage, which decreases the sensitivity and grain of the emulsion.

It is an object of this invention to provide a process of hardening photographic silver halide emulsions.

A further object resides in the provision of a hardening agent, which increases the sensitivity of the silver halide emulsion.

A still further object is the provision of an emulsion containing said hardening agent.

Still further objects will appear from the detailed specification following hereinafter.

It has been proposed to harden photographic silver halide emulsions with the aid of basicly substituted aldehydes and to simultaneously increase their sensitivity. This compensates the decrease suffered in sensitivity as well as in graination, which usually occurs during storing. To the aldehydes suitable according to this invention belong aliphatic aldehydes, containing a free or a substituted NH<sub>2</sub> group. In the latter case the amino groups may be substituted by alkyl radicals. But also such substituted aldehydes may be applied, which contain a ring substituent with a nitrogen atom in the nucleus. The following compounds serve as an example: amino-acetic aldehyde, aminodiacetic aldehyde, diethyl aminoacetic aldehyde, piperidinoacetic aldehyde,  $\beta$ -diethylamino propionic aldehyde and functional derivatives like aminoacetic aldehyde bisulfite and the respective oxime. The hardening agent may be added to the finished emulsion before casting. It may be applied in every phase during the manufacturing process of the emulsion, it may serve as preliminary bath before developing or be added to the developer itself. Needless to say these hardening agents like all others hitherto known may be applied to harden the emulsion layers after development, and to harden also other substances and structures influenced by aldehydes. In this case however the characteristics of the hardening agents, to increase simultaneously the sensitivity of the emulsion, have no practical effect.

## Example I

0.5 gram piperidino acetic aldehyde chlorine 55

hydrate is added to 1 kg. X-ray emulsion and cast in the usual way. The melting point is driven to 35° C. for the fresh emulsion, whereas the melting point for the corresponding test emulsion without hardening agent lies at 32° C. The increase in sensitivity accomplished by adding the hardening agent is very considerable. During storage the melting point increases to 46° C., but the sensitivity remains clearly above 10 the one of the not-hardened starting material.

## Example II

0.5 gram diethylamino acetic aldehyde is added to 1 kg. of an orthochromatic or panchromatic emulsion. The emulsion is cast onto films or plates in the usual way. The effect of the hardening agent towards the emulsion is the same as in Example I.

What we claim is:

20 1. A process of hardening photographic emulsions which comprises adding to a photographic silver halide gelatin emulsion an aliphatic amino-aldehyde selected from the group consisting of a compound corresponding to the following formulas



30 and



35 wherein R<sub>1</sub> and R<sub>2</sub> are selected from the class consisting of H and alkyl, R<sub>3</sub> and R<sub>4</sub> are alkylene and n stands for the number 1 and 2.

2. A process of hardening photographic emulsions which comprises adding to a photographic silver halide gelatin emulsion amino-acetaldehyde.

3. A process of hardening photographic emulsions which comprises adding to a photographic silver halide gelatin emulsion diethylamino-acetic aldehyde.

4. A process of hardening photographic emulsions which comprises adding to a photographic silver halide gelatin emulsion piperidino acetic aldehyde.

JOHANNES BRUNKEN.  
HANS FRICKE.  
GUSTAV WILMANNS.